

Dec. 27, 1927.

1,654,286

L. E. FROST

WOOD STRAIN INSULATOR

Filed March 14, 1921



Fig. 2.



Fig. 3.



WITNESSES:

L. F. Sonnemann.  
H. C. Bieman

INVENTOR

Leslie E. Frost.  
BY  
Wesley G. Barr  
ATTORNEY

Patented Dec. 27, 1927.

1,654,286

# UNITED STATES PATENT OFFICE.

LESLIE E. FROST, OF PITTSBURGH, PENNSYLVANIA, ASSIGNOR TO WESTINGHOUSE ELECTRIC & MANUFACTURING COMPANY, A CORPORATION OF PENNSYLVANIA.

## WOOD STRAIN INSULATOR.

Application filed March 14, 1921. Serial No. 452,198.

My invention relates to composite articles, more especially to composite wood strain insulators for use on trolley and transmission lines of relatively high-voltage 5 capacity and to a method of forming the same.

Heretofore, it was customary to employ kiln-dried hard woods, which were treated with asphaltum gums to make them moisture repellent, for insulators on relatively high-voltage transmission lines. It was very difficult to get uniform and deep impregnation in every instance and, because of this deficiency, such insulators frequently failed 10 in service because of the absorption of moisture.

As an improvement over this method, it has been proposed to first impregnate kiln-dried wood with paraffin and then impregnate it with a moisture-proof gum, the 20 object of this double impregnation being to obtain a deeper penetration of the impregnating materials, thereby obtaining greater uniformity in quality. This method, although more dependable than the former, 25 is somewhat complicated.

My invention obviates these difficulties, it being among the objects thereof to form strain insulators in an efficient and simple 30 manner.

It is a further object of this invention to form composite wood strain insulators which are moisture proof, which have a high dielectric strength, which are mechanically 35 strong and which will not deteriorate under varying atmospheric conditions.

In practicing my invention, I provide a body of hard wood, preferably maple, which is thoroughly dried by baking for approximately 40 twelve hours at 100° C. I then apply one coat of insulating varnish, such as spar varnish, which is hardened by baking in an oven. Next, the body is placed between the rotating centers of a lathe and a 45 coat of spar varnish is applied with a brush or in any other suitable manner. While the varnish is in a tacky or plastic condition, I wind a strip of cloth impregnated with a varnish, such as a copal gum and linseed oil 50 varnish, helically around the outer surface and then apply another coat of spar varnish on the surface thereof. This process is repeated until a suitable number of layers of treated cloth material has been formed and a 55 coating of spar varnish is applied. The

structure is then baked to harden the varnish. I then swage a metallic member or cap on each end of the insulating member, and, to further protect it, I apply a number of coatings of weatherproof paint. 60

In the accompanying drawings forming a part hereof and in which like reference characters designate like parts,

Figure 1 is a cross-sectional view of a wood strain insulator made in accordance 65 with my invention,

Fig. 2 is a sectional view thereof along the line II—II of Fig. 1, and

Fig. 3 is a sectional view of the insulator 70 along the line III—III of Fig. 1.

I provide a body of wood 1, preferably hard maple, which I thoroughly dry by heating for twelve hours at a temperature of 100° C. I apply a coating of spar varnish upon the surface 2 thereof and then 75 bake the varnish to harden it. The member 1 is mounted between the rotating centers of a lathe and another coating of spar varnish is applied and a strip of cloth impregnated with an insulating varnish is 80 wound helically along the surface 2, forming a layer 3, which is again coated with a layer of spar varnish and another layer of impregnated cloth is wound thereon. This 85 process may be repeated as many times as is desired, usually three or four layers being sufficient. I then apply a coating of spar varnish to the surface of the structure and subject the same to heat in an oven for a suitable length of time, to harden 90 the varnish, making the structure moisture proof. I further provide a pair of metallic members 4 and 5, which I swage on the tapered ends 6 and 7 of the body 1 and then apply a number of coatings of weatherproof paint to the insulator to further protect it against atmospheric conditions. 95

Although I have described a specific embodiment of my invention, it will be obvious to those skilled in the art that various modifications may be made therein without departing from the principles herein set forth. For instance, I may substitute any suitable insulating resins or varnishes, such as phenolic condensation products, casein, blood glues and the like for the spar or insulating varnishes. I may further swage the end members on the ends of the insulator before winding the treated cloth thereon or I may employ any number of 105 110

layers of cloth with alternating layers of varnish coatings.

It will be seen from the above description of my invention that wood strain insulators formed in this manner are highly moisture repellent and possess relatively high dielectric strength, one of the important advantages being that wood strain insulators made by this process are uniform 10 in quality and reliable in service.

I claim as my invention:—

1. A composite article comprising a body of wood having a layer of insulating varnish thereon and a plurality of alternate 15 layers of sheet insulating material and insulating varnish formed thereon.

2. A composite article comprising a body of wood having a plurality of coatings of insulating varnish and a plurality of layers 20 of sheet insulation material alternately formed on the surface thereof in the order named.

3. A method of forming composite articles which comprises providing a body 25 of wood, drying said wood by heating in

an oven, coating the outer surface thereof with a varnish, hardening said varnish by baking, applying another coat of varnish, winding a strip of fibrous material around said body of wood on said varnish while 30 plastic, applying a coat of varnish on said wound strip and baking to harden the surface.

4. A method of forming composite articles which comprises providing a body of 35 hard wood, drying said hard wood by heating in an oven at a temperature of 100° C., coating the surface thereof with an insulating varnish, hardening said varnish by baking in an oven, applying a coat of insulating 40 varnish, winding a strip of cloth around said body while the varnish is plastic, applying another coating of insulating varnish and another layer of cloth, and applying another coating of varnish and heat 45 hardening the same by baking.

In testimony whereof, I have hereunto subscribed my name this 28th day of February, 1921.

LESLIE E. FROST.